

# UNITED STATES PATENT OFFICE.

GEORGE L. KELLEY, OF GERMANTOWN, AND ALBERT H. MILLER, OF AMBLER, PENNSYLVANIA, ASSIGNORS TO THE MIDVALE STEEL COMPANY, OF PHILADELPHIA, PENNSYLVANIA, A CORPORATION OF PENNSYLVANIA.

## HIGH-SPEED-CUTTING-TOOL ALLOY.

1,258,227.

Specification of Letters Patent.

Patented Mar. 5, 1918.

No Drawing.

Application filed June 26, 1917. Serial No. 177,053.

*To all whom it may concern:*

Be it known that we, GEORGE L. KELLEY and ALBERT H. MILLER, citizens of the United States, residing at Germantown, county 5 of Philadelphia, and State of Pennsylvania, and Ambler, county of Montgomery, and State of Pennsylvania, respectively, have invented a new and useful Improvement in High-Speed-Cutting-Tool Alloys, of which 10 the following is a full, clear, and exact description.

The object of our invention is to provide an alloy suitable for use in the manufacture 15 of high speed cutting tools, and which, in addition to having in normal degree the qualities required for such tools, will give them in an especial degree the quality of toughness.

The use of zirconium as an element of 20 such an alloy has heretofore been known and its use, associated with a preponderating amount of nickel or cobalt, has been recommended in proportions varying from two to forty per cent. We have found, 25 however, that a superior product may be obtained if the quantity of zirconium be reduced to below what has heretofore been considered the minimum of efficiency provided there are associated with the zirconium 30 aluminum and silicon in certain minimum proportions substantially exceeding the proportion of zirconium.

The composition which we prefer comprises the following ingredients in the proportions specified:

|           |       |      |           |
|-----------|-------|------|-----------|
| Carbon    | ----- | .1   | per cent. |
| Nickel    | ----- | 86.4 | " "       |
| Aluminum  | ----- | 6.   | " "       |
| Silicon   | ----- | 6.   | " "       |
| Zirconium | ----- | 1.5  | " "       |

Corresponding proportions of the above ingredients, or part of the nickel alone, may be displaced by tungsten, which may be 45 added in proportions varying from 1 to 10 per cent.

The zirconium may vary from .5 to 2 per cent. A larger proportion of zirconium is not prohibitive, but where silicon and 50 aluminum are present in the required proportions, an excess of zirconium is without

benefit and may be harmful, whereas if a substantial proportion of silicon and aluminum is not present, an excess of zirconium produces an alloy having qualities different 55 from those sought.

While we prefer the proportions of aluminum and silicon specified, the proportions of each may range from 2 to 8 per cent. If, however, either the aluminum or 60 silicon is reduced to (say) two per cent. it is preferred not to reduce the proportion of the other. Thus, we have found that 2 per cent. of silicon and 6 per cent. of aluminum give substantially the same qualities as 2 per 65 cent. of aluminum and 6 per cent. of silicon. While, therefore, it would seem that these two metals are substantial equivalents, this is found not to be actually the case, because an entire elimination of either metal 70 and its entire replacement by the other produce an alloy that is notably inferior.

While we find that our improved alloy is especially adapted to the manufacture of high speed cutting tools, we do not intend 75 to confine ourselves to this particular use, inasmuch as it may be found serviceable for other purposes.

Having now fully described our invention, what we desire to claim and protect 80 by Letters Patent is:

1. An alloy for high speed cutting tools containing a preponderating amount of nickel, zirconium one-half to two per cent., and an amount of aluminum and silicon at 85 least double the amount of zirconium.

2. An alloy for high speed cutting tools containing a preponderating amount of nickel, zirconium one-half to two per cent., and aluminum and silicon each of the last 90 two metals constituting from 2 to 8 per cent. of the alloy.

3. An alloy for high speed cutting tools containing a preponderating amount of nickel, zirconium not less than .05 per cent., 95 and from 8 to 16 per cent. of aluminum and silicon.

In testimony of which invention we have hereunto set our hands at Philadelphia, on this 22d day of June, 1917.

G. L. KELLEY.  
A. H. MILLER.